

Patented Jan. 29, 1929.

## UNITED STATES PATENT OFFICE.

ROBERT E. WILSON, OF CHICAGO, ILLINOIS, ASSIGNOR TO STANDARD OIL COMPANY,  
OF WHITING, INDIANA, A CORPORATION OF INDIANA.

## AUTOMOBILE MOTOR COOLING OIL.

No Drawing.

Application filed April 21, 1925, Serial No. 24,883.

The present invention relates to improvements in automobile motor cooling oils. In accordance with the present invention a hydro-carbon oil product suitable for use 5 in the cooling of automobiles in place of water, solutions of salt, such as calcium chloride, alcohol mixtures, glycerine mixtures and the like is formed by a hydrocarbon oil product having a flash point of at 10 least 190° F., a viscosity below 45 sec. Saybolt at 100° F., and a boiling point range extending from about 400° F. up to about 600° F., or somewhat higher. A suitable oil for use 15 in accordance with this invention is one having a flash point of 200 to 210° F., a viscosity of 36 sec. Saybolt at 100° F., and a boiling point range of from 450° to 550° F.

The oils employed for automobile motor cooling in accordance with the present invention are capable of use in weather at 20 very low temperatures, as they do not solidify or reach high viscosities even at very low winter temperatures, nor is there any

substantial change in their characteristics during use. They flow freely, forming efficient cooling media, do not lead to fire danger and have substantially no injurious action upon the metallic and non-metallic parts forming the circuit for circulation for the cooling medium.

The oil may suitably be prepared by distilling crude or other suitable oil, subjecting the vapors thereof to an effective fractionation and selecting a relatively close cut having the specified properties.

I claim:

1. An automobile motor cooling oil consisting of a hydrocarbon oil having a flash point not less than 190° F., a viscosity below 45 sec. Saybolt at 100° F., an initial boiling point not below 400° F.

2. An automobile motor cooling oil having a flash point of 200 to 210° F., a viscosity 36 sec. Saybolt at 100° F., and a boiling point range of 450 to 550° F.

ROBERT E. WILSON.